

A. R. TERRY.

Coating Gas Retorts.

No. 11,142.

Patented June 20, 1854.



# UNITED STATES PATENT OFFICE.

ADRIAN R. TERRY, OF DETROIT, MICHIGAN.

## COATING GAS-RETORTS.

Specification of Letters Patent No. 11,142, dated June 20, 1854.

*To all whom it may concern:*

Be it known that I, ADRIAN R. TERRY, of the city of Detroit, county of Wayne, State of Michigan, have invented a new mode of 5 protecting gas-retorts or iron—that is, the retorts commonly used for manufacturing carbureted hydrogen gas from coal, wood, oil, resins, &c., for lighting and culinary purposes—from the destructive action of the 10 fire and also from the action of the sulfur and other constituents of the materials used in making gas, which have a strong affinity for iron at a high heat. By the same method of protection, gas retorts made of 15 boiler or other thick sheet iron may be economically substituted for the more expensive gas retorts of cast iron. And I do hereby declare that the following is a full and exact description thereof.

20 The gas-retorts now generally used are of cast-iron, and the continued red heat, necessary to generate carbureted hydrogen gas, produces rapid oxidation on the outside; also the access of the atmospheric air to the 25 inside of the retort during the process of removing the coke, cleaning the retort from ashes, and recharging it with coal or other materials, produces rapid reduction of temperature, and is according to known facts 30 productive of changes in the arrangement of the molecules of the iron injurious to its strength; the action of the sulfur, too, contained in bituminous coal and some other products of its destructive distillation, as 35 well as the products of the same process from wood, and other substances used for making carbureted hydrogen gas, for lighting, culinary, and other purposes, have a powerful action on the inside of the retort, 40 uniting with the iron and making brittle and friable compounds, which by cracking and scaling off, decrease the strength of the iron. All of which causes unite to destroy 45 gas retorts, in a period extending from eight to fourteen months. There is another loss occasioned by the rapid cooling of the iron retorts, during the process of cleaning and charging; and that is in the quantity of gas 50 manufactured in a given time. If the temperature is but slightly lowered, during the time of cleaning and charging, it is obvious 55 that the evolution of gas will begin soon after the introduction of the new charge, but if a great loss of heat takes place during the process, the evolution of gas will be much

retarded; this I consider a point of importance in my invention.

To obviate these various disadvantages is the object of my invention and this object I propose to attain in the following manner.

60 I envelop the retort from the flange at the mouth, to the rear or back end, on the outside, with a net work of annealed iron, steel, copper or brass wire or its equivalent metallic cloth: the wires to be so applied that 65 they shall cross each other at different angles and in different directions, so that they may form meshes of about three-eighths of an inch, more or less in diameter. If wire-cloth be employed the meshes should be 70 about three eighths of an inch in diameter; in both methods the wire used should be from number eighteen to number twenty-two.

75 A compound of common blue clay (such as is used for making coarse earthenware) silicious sand, and borax or some other alkaline, earthy or metallic flux or its equivalent, in the ratio say of clay 30 parts, sand 66 parts, and flux 4 parts, by weight, tempered with water to the consistence of thin mortar, should then be applied, over the wire net work, in a stratum about an eighth of an inch thick and suffered to dry in the air, sheltered from rain and frost. The 80 quantity of sand must be increased or decreased according to the quality of the clay; the rule being to add as much sand as possible, without impairing too much the adhesiveness of the compound. The quantity of 85 flux must be varied, according as one or another is employed; the object being to make a covering which will become semivitrified at the heat used for making carbureted hydrogen gas. The above proportion of flux 90 is based on the employment of borate of soda or borax.

95 As soon as the first coat has attained a moderate degree of firmness, another coat of about half the thickness is applied, and when this is dry enough not to yield to pretty strong pressure with the finger, another network of wire is applied, and again two coatings of the composition. From five to eight networks of wire are to be applied, and, of course, from ten to sixteen strata of the composition. Each coating should be 100 brushed over, when partially dry, with a strong solution of borax or other alkaline flux or its equivalent. The aggregate thick- 105 110

ness of the strata or coatings may vary from three-fourths of an inch to an inch and a half, according to the size of the retort, the heat to be employed &c.; the thicker the covering is, the less will be the heat lost during cleaning and charging.

After the coating is thoroughly dry a semi-vitrifiable composition, consisting of clay potash or soda and oxid of lead or litharge, in the following proportions, clay ten parts, potash or soda ten to fifteen parts, silicious sand fifty parts, and litharge thirty parts, tempered with water to the consistency of thick cream, should be applied three or four times with a brush over the surface of the outer coating. Suffering it to dry, after each application. This concludes the preparation of the outside of the retort.

The inside of the gas retort is to be protected from the action of the sulfur, &c., as before specified, by a composition similar to that described above as being put on over the last stratum or coating of the composition on the outside of the retort, viz, clay, potash or soda, silicious sand, and litharge. The clay in this should be in rather larger proportion to make it more adhesive.

This composition should be put on with a brush in successive coats over the whole internal surface of the retort.

Each coating should be suffered to become thoroughly dry before another is applied; in this way the composition will adhere firmly to the inside surface of the retort, and will become vitrified when heated in the gas-oven, protecting the iron from the action of the sulfur, &c., of the materials as specified above.

The proportions of the materials for the interior coating may be varied as further experience shall dictate.

The interior coating may be renewed from time to time without cooling the retort, in the following manner: A dry powder of the following materials, in these proportions, crystallized carbonate of soda twenty-nine parts, oxid of lead (litharge) thirty parts, and pure silicious sand sixty parts by weight,

is thrown into the retort and made to come in contact with all parts of its interior surface. The action is as follows: The large quantity of water contained in the carbonate of soda causes the materials to undergo a sort of watery fusion, on coming in contact with the red-hot iron, and adhere strongly to it, where they soon become vitrified.

No further care to prevent the cracking of the external and internal coatings is necessary than the care always used in gradually heating up gas-retorts for the first time.

Having thus fully described the method of treating gas-retorts in which my invention consists, I shall merely refer to the accompanying drawings, which represent a perspective view of an ordinary gas-retort, the parts A and B showing the manner of wrapping, and of applying the composition.

I am aware that different means have been used to prepare gas-retorts which should not be liable to the disadvantages of the ordinary iron and clay gas-retorts, and that retorts for making potassium and for other purposes have been wrapped and coated with clay, but that was for a higher heat continued but a short time, while the peculiarity of my composition and method of application is that it is calculated to withstand a comparatively moderate heat for a long time; and should slight cracks take place on first heating up, the semi-vitrification of the composition closes them. The number of strata or coatings is a matter of much importance as a check or crack in one stratum is found by experience not to extend to the one next below it.

What I claim as my invention, and wish to secure by Letters Patent is:

The application to gas retorts of a coating which consists of a series of layers or lamineæ of luting and metallic wrapping substantially as specified.

ADRIAN R. TERRY.

Witnesses:

A. W. BOWMAN,  
N. CALLAN.